

# UNITED STATES PATENT OFFICE.

HANS TOEPFER, OF NEW YORK, N. Y., ASSIGNOR TO THE GRASSELLI CHEMICAL COMPANY, OF CLEVELAND, OHIO, A CORPORATION OF OHIO.

## PROCESS OF DYEING.

1,417,869.

Specification of Letters Patent. Patented May 30, 1922.

No Drawing.

Application filed August 4, 1921. Serial No. 489,849.

To all whom it may concern:

Be it known that I, HANS TOEPFER, a citizen of Germany, residing at New York city, in the county of New York and State of New York, have invented certain new and useful Improvements in Processes of Dyeing, of which the following is a specification.

It is a general practice to treat the animal fibres dyed with the so-called mordant colors with chromium salts in order to obtain the desired shades and fastness properties. In such dyeing processes the chromium salts can be applied to the animal fibres before dyeing, they can be added to the dye bath, or the dyed goods can be after treated with chromium salts. With the exception of copper salts which are used in a few instances, no other salts of heavy metals have ever found a practical application for the treatment of dyed animal fibres.

I have now found that the shade and fastness of animal fibres, that is to say wool and silk, dyed with azo colors having as one component ortho-amidophenol with one or more nitro-groups in the same benzene nucleus can be greatly improved by using in conjunction therewith a cobalt salt. This may be done either by applying the dyestuff after the fiber has been mordanted with cobalt salts; or by adding cobalt salts to the dye bath; or preferably by after treating the dyed fibre with cobalt salts.

As examples of such nitro-ortho-amido-phenol azo dyestuffs I may mention:

(1) The combination of picramic acid and naphthionic acid described in Schultz-Julius #91:

(2) The compound



45 described in U. S. Patent 936,321, Oct. 12, 1909.

(3) The compound



50

described in U. S. Patent 843,077, Feb. 5, 55 1907.

(4) Or the compound



60

65

described in U. S. Patent 1,159,375, Nov. 9, 1915, but I wish it understood that our invention is not limited to the above mentioned 70 dyestuffs.

In order to illustrate more fully the new process, the following examples are given:

Example 1.—100 parts of wool are dyed in the usual way with 2 parts of the dyestuff prepared by coupling naphthionic acid with diazotized picramic acid (Schultz-Julius #91); 10 parts of Glauber's salt and 2 parts of acetic acid are added and the bath is heated to boiling for  $\frac{3}{4}$  of an hour.  $\frac{1}{2}$  part 80 of sulfuric acid is then added in order to exhaust the dye bath and boiled for 15 minutes longer; thereafter 2 parts of cobalt sulfate, or an equivalent amount of cobalt chlorid or cobalt acetate are added and boiled 85 for  $\frac{1}{2}$  hour. The dyed goods are rinsed. A green shade, very fast to light is obtained. It is much brighter than the one obtained by after treating the same dyeings with other metal salts, e. g., chrome. This shade has 90 further the advantage of being as brilliant under artificial light as by daylight.

Example 2.—100 parts of wool are mordanted with 3 parts of cobalt chlorid and 1

part of acetic acid, boiled for 1 hour and rinsed. The goods are entered cold into a dye bath containing 2 parts of the dyestuff prepared according to U. S. Patent 843,077 of Feb. 5, 1907, and 2 parts of acetic acid, heated to the boiling temperature, boiled for 1 hour and rinsed. A light fast blue shade is obtained.

*Example 3.*—A dye bath is prepared from 10 60 parts of water, 2 parts of cobalt chloride and 2 parts of the dyestuff prepared according to U. S. Patent 936,321 of Oct. 12, 1909. 100 parts of wool are entered at 140° F. The dye bath is brought up to the boiling temperature, boiled for  $\frac{1}{2}$  hour, then 2 parts of

acetic acid are added and boiled for  $\frac{3}{4}$  hour longer. The dyed goods are rinsed. A dark brown shade is obtained which compares very favorably in light fastness to the brown obtained in a bichromate bath.

20

I claim:—

1. In the art of dyeing animal fibres, the process comprising using cobalt salts in conjunction with azo dyestuffs derived from nitro-ortho-amidophenols.

2. Process according to claim 1 in which the cobalt salts are applied to the dyed fibre.

In testimony whereof, I affix my signature.

25

HANS TOEPPER.